

# UNITED STATES PATENT OFFICE.

CHARLES F. ALIESKY, OF BROOKLYN, NEW YORK.

## ENAMELING JEWELRY.

SPECIFICATION forming part of Letters Patent No. 240,876, dated May 3, 1881.  
Application filed April 6, 1881. (Specimens.)

*To all whom it may concern:*

Be it known that I, CHARLES F. ALIESKY, of Brooklyn, in the county of Kings and State of New York, have invented certain new and useful Improvements in Enameling Jewelry, of which the following is a specification.

This invention is designed to produce on chased or engraved articles of jewelry made of silver, gold, or other metals a permanently-adhering coating of enamel, through which the chased or engraved designs are clearly visible, so as to increase the artistic effect of the same and furnish thus more elegant and more permanent articles of ornamental jewelry.

15 Heretofore, in enameling jewelry, the enamel was laid on in thick layers, which, to prevent cracking, had to be laid on at both sides of the metal, so as to counteract to some extent the difference of contraction between the metal and 20 the enamel. Owing to the thick layer of enamel employed, it has not been possible to bring out finely-chased or engraved designs in enamel, and consequently it could not be used for ornamenting chased or engraved articles.

25 I have succeeded in making enameled articles of jewelry in which the enamel is laid on in thin layers like glazing, so that even the most minutely chased or engraved portions are brought out; and the invention consists, first, 30 in covering the surface of the chased or engraved article of jewelry with a translucent layer of enamel, and burning in this layer, then laying upon the translucent enamel one or more layers of colored enamel and burning them in 35 at one or more burnings, according to the colors employed.

In following out my improved method of enameling jewelry, the surface of the same is first chased or engraved to the proper design.

Upon the chased or engraved surface is now 40 laid on, with a brush, a thin layer of translucent enamel, which is burned in in the muffle, in the usual manner. Upon this translucent coating or layer of enamel one or more layers of colored enamel are laid on and burned in, either 45 by one or more burnings, according to the character and blending of the colored enamels employed. The thin layers of enamel do not cover up the chased or engraved design, but render the same visible in all its details, the colors 50 even serving to heighten the beauty and artistic effect of the same, so that jewelry of highly improved appearance and great permanency is obtained, as the enamel is not liable to crack, but adheres firmly to the surface. 55

Having thus described my invention, I claim as new and desire to secure by Letters Patent—

1. The method herein described of enameling jewelry, consisting, first, in coating chased and 60 engraved articles of jewelry with a thin layer of translucent enamel and burning in the same, next laying on one or more coatings of colored enamel and fixing the same by one or more burnings, substantially as set forth. 65

2. As a new article of manufacture, chased or engraved jewelry covered by a layer of translucent enamel, and by one or more layers of colored enamel, substantially as specified.

In testimony that I claim the foregoing as 70 my invention I have signed my name, in presence of two witnesses, this 5th day of April, 1881.

CHARLES F. ALIESKY.

Witnesses:

PAUL GOEPEL,  
CARL KARP.